

# UNITED STATES PATENT OFFICE.

FERNAND GEO. WHITE, OF MERIDEN, CONNECTICUT.

## METHOD OF PRODUCING COAL-TAR PAINT.

1,396,674.

No Drawing.

Application filed August 19, 1921. Serial No. 493,725.

Specification of Letters Patent. Patented Nov. 8, 1921.

To all whom it may concern:  
Be it known that I, FERNAND G. WHITE, a citizen of the United States, residing at Meriden, in the county of New Haven and State of Connecticut, have invented a new and useful Improvement in Methods of Producing Coal-Tar Paint; and I do hereby declare the following to be a full, clear, and exact description of the same.

10 My invention relates to an improved method of producing, from the raw coal tar derived from the distillation of gas coals, or coals of high volatile content, a paint particularly designed for use in dressing cloth or leather automobile tops, but also adapted to be used for kindred purposes, the object being to produce, at a low cost, a dressing of superior flexibility, preserving quality, and permanence, as well as providing an attractive finish, whereby faded tops may be restored to a fine appearance.

In carrying out my invention, I take a quantity of the raw coal tar resulting from the distillation of what is known 25 in the market as "gas coals," which are coals of high volatile content. The raw tar is placed in a suitable still in which it is subjected to constant agitation, by the injection of air or by some mechanical stirring apparatus, the agitation of the tar being continued throughout the process. Heat is applied under the container of the still and the tar gradually heated until it reaches a temperature of substantially 160° F. At this 30 temperature, the water content of the tar will begin to be discharged from the coil of the still. The temperature of the still is now raised very slowly to a temperature of substantially 180° F. and may even be raised to 35 190° F. Particular care should be taken to raise the temperature of the tar in the container from 160° F. to 180° F. or more very slowly, since otherwise the tar will boil over and be discharged through the coil with the 40 condensed water. At least one hour should be allowed for raising the temperature of the tar from 160° F. to 180° or 190° F. The still should thereafter be run at a temperature of 45 180° F. to 190° F. until the emulsion which comes from the coil is about three parts of light tar oil to one part of water. The temperature of the still is now slowly raised until a temperature of substantially 310° F. is reached; this temperature should not exceed 50 325° F. or thereabout, since above this temperature the heavy oil will begin to go

over, in which case the tar in the container will be so changed in character that it cannot, subsequently, be used in the production of my improved paint.

Under the process described, only the light oil contained in the raw tar is removed, leaving substantially all of the heavy tar oil in the tar, but the ammoniacal content of the raw tar is driven off during the described 65 distilling operation, so that substantially no ammonia remains in the dehydrated tar in the container of the still.

The fire is now drawn and the tar remaining in the container allowed to cool to a temperature of from 100° to 125° F., the object being to keep the tar fluid enough to be readily stirred, but not hot enough to cause explosions.

Practically all the tar oil which passes 75 off with the water during the operation described is lighter than water, though very small quantities of heavier-than-water oil may come over with the water and lighter oil, depending on the raw tar used and on 80 the temperatures reached during the distilling operation. Such lighter-than-water tar oil is then poured into the dehydrated tar remaining in the container and stirred into it until the entire body of tar is reduced 85 to the consistency of thin paint. It is to be understood, however, that the amount of light tar oil produced from the distillation of any given volume of raw tar will not be sufficient to thin the dehydrated tar in the 90 container to the consistency of paint, but other light tar oil must be added to the amount driven off during the distillation of any given amount of tar. I might here explain that any tar oil lighter than water 95 may be used in this thinning operation.

The paint produced by the above process is then ready for use and is applied by a brush to cloth and leather for automobile tops, for which it acts as a preservative and binder, imparting a fine finish and fadeless color; also it is practically permanent as to its flexibility.

I do not limit myself to the exact temperatures herein given, my invention consisting 105 broadly in a process characterized by adding the lighter-than-water tar oil to coal tar, from which the water and lighter-than-water oil has been removed.

I claim:

1. An improved method of producing an elastic, preservative dressing for cloth,

leather and kindred materials, consisting in distilling raw coal tar to drive off its water and lighter-than-water oil, then cooling the dehydrated tar and reducing it to the thinness of paint by the addition to it of tar oil lighter than water.

2. An improved method of producing an elastic, preservative dressing for cloth, leather and kindred materials, consisting in 10 placing raw coal tar in a still and raising it to the temperature at which the discharge from the coil is substantially one part of water and three parts of lighter-than-water oil, then continuing the process of distilla-

tion until the temperature of the still reaches 15 substantially  $310^{\circ}$  F., then arresting the distilling operation and allowing the distilled tar to cool, and then adding a sufficient amount of tar oil lighter than water to reduce the consistency of the mass to that 20 of thin paint.

In testimony whereof I have signed this specification in the presence of two subscribing witnesses.

FERNAND GEO. WHITE.

Witnesses:

EMMA A. WHITE,  
EARL F. WHITE.